

1

**3,169,071**  
**COATING COMPOSITION**

Harry Hochman, Woodland Hills, Calif., assignor to the United States of America as represented by the Secretary of the Navy

No Drawing. Filed June 6, 1961, Ser. No. 115,270

1 Claim. (Cl. 106—15)

(Granted under Title 35, U.S. Code (1952), sec. 266)

The invention described herein may be manufactured and used by or for the Government of the United States of America for governmental purposes without the payment of any royalties thereon or therefor.

This invention relates generally to coating compositions for wooden structures in a marine environment and particularly to hydrocarbon derivatives containing bactericidal or bacteriostatic components.

The use of wood for marine structures adjacent to and in the waters of rivers, lakes and oceans extends from antiquity to the present day; the availability of metals and concrete notwithstanding. Concomitant with the use of wood, its marine biological deterioration has been a continuing problem for the same length of time. Unprotected wood in contact with water soon becomes honeycombed with the burrows of marine wood boring animals and its imminent failure is ever present. A good sized pile may be destroyed in as short a time as six months. Treated wood lasts longer, but all too often the wood borers somehow gain entrance and their destructive activities may begin long before the serviceable life of the boat, float, pile, or dock should be ended.

The extent of the problem can be expressed most dramatically in terms of financial losses. It is estimated that American losses run annually to some five hundred million dollars. Undoubtedly corresponding and proportionate losses are experienced abroad. Such losses testify to the fact that present methods for protecting wood from deterioration in sea water, particularly, are either far from effective or that there is somewhere a failure in their successful application.

Many compositions for preserving and protecting wood in a marine environment have been proposed in the past. Of them all, creosote, whether derived from coal or wood tar, has been found to be one of the most effective deterrents to such biological infestation, particularly from the standpoint of availability, cost, and ease of application.

Creosote treated wood serves for long periods of time in many harbors. In other harbors, however, even creosoted wood has a relatively short service life. In comparatively cold water harbors, creosote treated piling may last for 30 years or more. In warm water harbors, however, such treatment may not protect the wood for more than a few years. Thus, it has been found that the average service life of creosoted piling in Los Angeles Harbor is about 15 years; Pearl Harbor, Hawaii, 8 years; and at Key West, Florida, about 5 years.

It has been assumed, previously, that creosote loses its effectiveness because it is more readily leached out of the wood in the warm water harbors than it is in the cold water harbors. While it is probably true that leaching does remove a considerable fraction of the creosote from the wood after a long period of exposure in a marine environment, it has been found that creosote treated wood that has been leached for 12 years in certain warm water harbors is still toxic enough to repel the attacks of marine borers. Since marine borers can destroy a creosoted pile in 5 years and creosote treated wood leached for the equivalent of 12 years is still toxic to these borers, leaching per se cannot be the sole method, indeed it may not be the principal method, by which creosote loses its effectiveness.

2

Examination of sections of creosoted piling that has been exposed in Port Hueneme, California, harbor for 15 years revealed that although the surface of the piling was still black with creosote, the surface impregnated wood was no longer toxic to marine borers. The creosote, itself, extracted from the surface of the pile was relatively non-toxic to borers. The creosote present in the wood below the surface was more toxic to borers and toxicity increased with depth until creosote taken from the wood two inches below the surface was found to be as toxic as fresh creosote. When that portion of the pile above the high water mark was examined, the surface creosote was still as toxic as fresh creosote. This evidence shows, conclusively, that in addition to the leaching of some of the preservative from the wood in the sections below the water line, another mechanism, a toxic destroying or modifying mechanism, was also active in decreasing the effectiveness of creosote below the water line.

In all the various harbors investigated, a varying quantity of bacteria have been found that can live on fully creosote treated wood. It is believed that it is the activity of these bacteria which, after a period of time, so alters creosote that its toxicity to marine boring organisms decreases. It is further believed that the rate of decrease in toxicity of creosote by the action of these bacteria can be greatly reduced by the incorporation of an effective bactericide or bacteriostatic compound into the creosote or by impregnating the wood separately by bactericidal compound followed by the standard impregnation with creosote.

If the bactericidal or bacteriostatic agent is soluble in organic solvents such as creosote, it would be of advantage to incorporate it into the creosote and use the entire solution as a single unit for the impregnation of the wood being treated. If the added agent is not soluble in creosote or cannot be successfully compounded therewith to produce a homogeneous fluid, the agent may be impregnated into the wood first, using an appropriate solvent as a carrier, and, following this treatment and subsequent drying of the wood, a second impregnation is carried out forcing the creosote into the wood to the depths desired. Obviously, the advantage of using such bactericidal or bacteriostatic agents with creosote is that by controlling the population of creosote tolerant bacteria, the original toxicity of creosote to marine boring organisms is prolonged indefinitely. Should the added agent be of a kind that is also attacked by the environment, it will still prolong the original effectiveness of the creosote and will decrease the rate by which creosote becomes ineffective. In this manner, the service life of creosoted timbers will be greatly increased even in those bacteria-infested harbors where, heretofore, their surface life has been relatively short.

Among the types of bactericides and bacteriostatic agents that have been found effective are metal compounds such as copper, zinc, mercury, and silver salts; metallo-organic derivatives such as organic mercuric compounds; triphenylmethane dyes such as malachite green and crystal violet; phenols and halogenated phenols such as pentachlorophenol; quinones such as methyl naphthoquinone; amines such as naphthylamines and acridine; quaternary ammonium compounds such as alkyl trimethyl ammonium and others, some of which will be mentioned hereinafter. It should be noted here that the choice of such bactericides or bacteriostatic agents is limited only by its solubility, toxicity, availability and economy. The most potent agent may not be the most advantageous when these factors are taken into consideration. The design service life of the wooden structure to be built is also an important factor.

In keeping with the philosophy and theory of my inven-

tion, i.e., the prolongation of the toxic effects of creosote when applied to wood structures exposed to a marine environment by controlling the attacks of creosote tolerant and creosote destroying bacteria, the following effective preservative methods and materials are set forth:

(1) The wood is first treated with an aqueous solution of copper sulphate containing between 1 and 10% copper and then, after drying, is impregnated with creosote to standard retentions.

(2) Methyl naphthoquinone is dissolved in creosote to produce solutions containing between 1 and 10% of the methyl naphthoquinone. The resulting solution is then impregnated into the timbers as a single treatment.

(3) Materials which are insoluble in creosote, such as copper sulphate, can be first converted into a copper chelate or oil soluble salt. This chelate or salt is then dissolved into the creosote to form a solution containing 1 to 10% of copper which solution is used to impregnate the wood. An example of a copper chelate that is soluble in creosote is copper oxinate. This was prepared by adding a solution of 13.1 g. of copper sulphate penta hydrate (0.062 mole) in 250 ml. of methanol to a solution of 36.4 g. (0.25 mole) of 8-hydroxyquinoline (oxine) in 400 ml. of methanol. The copper oxinate crystallized out as needles.

Similarly, zinc oxinate was prepared from 4.4 g. (0.02 mole) of zinc acetate in 150 ml. of methanol and 17.5 g. (0.12 mole) of oxine in 175 ml. of methanol.

(4) Another copper salt soluble in creosote may be obtained by converting copper sulphate to a higher fatty acid salt. Thus, a copper oleate was prepared by dissolving 12.5 g. (0.05 mole) of copper sulphate in 150 ml. of methanol and adding this solution to a solution of 30.0 g. of oleic acid in 750 ml. of methanol. To the resulting solution, an equal volume of water was added with a sufficient quantity of a 10% sodium hydroxide solution to raise the pH above 7.0. The copper oleate separated out as a blue solid which was then filtered.

(5) Materials which are insoluble in creosote may also emulsify to produce homogeneous liquids capable of being impregnated in wood in a single operation. For example, malachite green oxalate is insoluble in creosote. If it is first triturated with an emulsifying agent such as sorbitan trioleate, it can be readily incorporated into creosote. Thus, if a 1% solution of malachite green in creosote is desired, 1 g. of malachite green oxalate is triturated with 0.1 to 5 g. of sorbitan trioleate and then added to 100 ml. of creosote.

Having thus described my invention, its practice, and the formulation of various bactericidal and bacteriostatic agents that may be employed therewith, I do not intend to be limited thereby except as such limitations may be included in the scope of the appended claim wherein,

I claim:

A preservative composition for impregnating wooden structures designed for installation in a marine environment consisting essentially of creosote and a bactericide for creosote-tolerant, creosote-attacking bacteria, said composition consisting of 90-99% creosote and 1-10% bactericidal agent selected from the group consisting of creosote soluble zinc oxinate, malachite green oxalate, and malachite green oxalate after trituration with sorbitan trioleate, an emulsifying agent.

#### References Cited by the Examiner

##### UNITED STATES PATENTS

|           |       |                  |          |
|-----------|-------|------------------|----------|
| 1,690,390 | 11/28 | Williams et al.  | 106-15   |
| 2,296,401 | 9/42  | Perkins          | 106-15   |
| 2,561,380 | 7/51  | Kalberg          | 106-15 X |
| 3,065,087 | 11/62 | Goldstein et al. | 106-15   |

MORRIS LIEBMAN, Primary Examiner.

JOSEPH REBOLD, ALEXANDER H. BRODMERKEL,  
Examiners.